

Nov. 18, 1969

A. I. BACKSTROM ET AL

3,479,181

PROCESS FOR THE PRODUCTION OF BIMETALLIC MATERIAL WITH HIGH  
RESISTANCE TO TRANSCRYSTALLINE STRESS CORROSION  
IN A CHLORIDE ENVIRONMENT

Filed Feb. 14, 1968

3 Sheets-Sheet 1

FIG.1



INVENTORS.

ARNE IVAR BACKSTRÖM,  
STURE HENRIKSON &  
PER ERIK LEVIN

BY

*Brunbaugh, Free, Graves & Dorothea*  
their ATTORNEYS.

Nov. 18, 1969

A. I. BACKSTROM ET AL

3,479,181

PROCESS FOR THE PRODUCTION OF BIMETALLIC MATERIAL WITH HIGH  
RESISTANCE TO TRANSCRYSTALLINE STRESS CORROSION  
IN A CHLORIDE ENVIRONMENT

Filed Feb. 14, 1968

3 Sheets-Sheet 2

FIG. 2



INVENTORS.

ARNE IVAR BACKSTRÖM,  
STURE HENRIKSON &  
PER ERIK LEVIN

BY

*Brumbaugh, Frey, Graves & Donohue*  
their ATTORNEYS.

Nov. 18, 1969

A. I. BACKSTROM ET AL  
PROCESS FOR THE PRODUCTION OF BIMETALLIC MATERIAL WITH HIGH  
RESISTANCE TO TRANSCRYSTALLINE STRESS CORROSION  
IN A CHLORIDE ENVIRONMENT

3,479,181

Filed Feb. 14, 1968

3 Sheets-Sheet 3

FIG.3A



FIG.3B



INVENTORS.

ARNE IVAR BACKSTRÖM,  
STURE HENRIKSON &  
PER ERIK LEVIN

BY

*Brumbaugh, Free, Graves + Donohue*  
their ATTORNEYS.

1

3,479,181

PROCESS FOR THE PRODUCTION OF BIMETALLIC MATERIAL WITH HIGH RESISTANCE TO TRANSCRYSTALLINE STRESS CORROSION IN A CHLORIDE ENVIRONMENT

Arne Ivar Backstrom, Sture Henrikson, and Per Erik Levin, Avesta, Sweden, assignors to Avesta Jernverks Aktiebolag, Avesta, Sweden, a Swedish joint-stock company

Filed Feb. 14, 1968, Ser. No. 705,490

Claims priority, application Sweden, Feb. 16, 1967,  
2,168/67

Int. Cl. C22c 33/02; B22f 1/00

U.S. Cl. 75—212

5 Claims

ABSTRACT OF THE DISCLOSURE

A process for the production of bimetallic austenitic stainless steel alloys having a resistance to transcrystalline stress corrosion in a chloride environment comprises plating an austenitic stainless steel in powder form with nickel, or nickel in combination with other corrosion resistant metals, in layers virtually coating each powder grain. The powder material is then heated to sinter it and is densified and stretched, such as by rolling, forging or extrusion such that the layers coated onto the powdered grains form corrosion impeding barriers oriented primarily in planes coinciding with the tensile stresses imposed on the material.

The normal types of austenitic chromium-nickel and chromium-nickel-molybdenum steel may, under certain conditions, be affected by so-called transcrystalline stress corrosion.

The corrosion attacks usually take the form of cracks which rapidly force their way deeper and deeper into the material, often breaking through entirely.

Transcrystalline stress corrosion will occur under the combined effect of the following factors:

(1) Tensile stresses. These may be residual, conditional on the design (resulting from welding, bending, machining, etc.) or have an operational basis (from pressure or temperature). The sensitivity rises with an increasing tensile stress. It is difficult to indicate the lowest stress which causes stress corrosion, since the sensitivity is also controlled by other factors. If the latter are severe, however, a stress corresponding to half the tensile stress limit at the temperature in question is sufficient to cause the formation of cracks.

(2) Specific corrosion media. The most common materials causing stress corrosion are chlorides, such as KCl, CaCl<sub>2</sub>, NaCl and MgCl<sub>2</sub>. In practice these chlorides are present in varying contents both in natural cooling water and in special cooling media. The sensitivity to stress corrosion increases with increasing chloride content. It is impossible, however, to indicate any threshold values below which the respective steel qualities are insensible owing to the risk for a local concentration in practical operation of contents no matter how low (e.g. by the evaporation of water).

(3) Temperature. The stress corrosion caused by chlorides is very rare below 40–50° C. However, the sensitivity increases considerably with increasing temperatures, a circumstance which is reflected by the chloride contents required to cause the stress corrosion. The chloride contents are the absolute contents in a water solution where no concentration takes place, thus achieved in ideal conditions during laboratory tests. For a steel with 18 percent chromium and 8 percent nickel and at 100° C. this content lies at about 50,000 p.p.m. (5 per-

2

cent) Cl, but at 150° C. and corresponding overpressure it is as low as 10 p.p.m.

(4) The redox potential of the solution. During laboratory tests it has been proved that the potential at which the steel sets in a chloride solution according to the redox potential in this solution is of decisive importance for stress corrosion. As a matter of fact stress corrosion seems to occur within a relatively limited potential range, about 30 mv, which is characteristic for each type of steel and is higher the more alloyed the steel is. Below this range of potential a cathodic protection of 100 percent is obtained.

(5) Composition of the steel. Nickel is the alloying element which most effectively reduces the sensitivity to stress corrosion. However, about 40 percent is required if this type of corrosion is entirely to be prevented. Chromium, silicon, molybdenum and copper may also increase the corrosion resistance to a certain extent.

It would seem obvious from what has been referred to above that a high nickel content is the most effective way to reduce or prevent stress corrosion. However, the nickel content must be maintained at a level of about 40 percent which, as a matter of fact, means that one cannot any longer talk about stainless steel but must instead refer to nickel alloys since the nickel content is higher than the iron content. As examples of commercial nickel alloys which are resistant to stress corrosion the following may be mentioned:

|               | Percent |       |       |       |      |       |
|---------------|---------|-------|-------|-------|------|-------|
|               | Ni      | Cr    | Mo    | Cu    | Mn   | Fe    |
| Mineral type: |         |       |       |       |      |       |
| I-----        | 40      | 21    | 3.0   | 1.75  | 0.60 | 33    |
| II-----       | 172     | 14-17 | ----- | 0.7   | 1.0  | 6.10  |
| III-----      | 199     | ----- | ----- | 0.25  | 0.35 | 0.40  |
| IV-----       | 163     | ----- | ----- | 28-34 | 2    | ----- |

<sup>1</sup> Minimum.

However, all the above alloys are expensive, mainly owing to the comparatively high nickel price.

The object of the present invention is to arrive at a process for the production of bimetallic austenitic stainless steel alloys with a high resistance to transcrystalline stress corrosion in a chloride environment and mainly characterized in that austenitic stainless steel powder is plated with nickel, if desired in combination with other metals, in layers practically coating each powder grain and where the said layers form corrosion-impeding barriers mainly orientated in planes coinciding with the tensile direction, after the powder material has been subjected to heat treatment as well as densifying and stretching by means of plastic shaping, such as rolling, forging or extrusion. The powder material is in that manner transformed into solid material in the shape of e.g. sheet metal, strips, bars or pipes. By stretching the material in the working process one obtains barriers relatively evenly divided in the basic material and orientated in the tensile direction. The distance between the barriers is determined by the rate of reduction in the working process and the particle size while the thickness of the barriers is further determined by the amount of metal added and the scope of the diffusion. The composition of the barriers depends on the composition of the plating, on the diffusion within the barriers and between these and the basic material, and finally on the composition of the basic material.

The heat treatment could appropriately be conducted at a temperature between 950 and 1300° C. The heat treatment may be conducted separately or be coincident with the heat treatment which usually takes place prior to the plastic working.

The process makes possible considerable saving of expensive alloying metals, especially nickel, since only a small part by weight is required of the amount which would be required if a homogeneous material with a composition identical to the barrier material were to be produced.

The present invention is further illustrated by the following examples, reference being simultaneously made to the attached drawings, where:

FIG. 1 shows a micrograph of a type of steel according to the present invention, magnified 150 times,

FIG. 2 shows schematically the diffusion process in a type of steel according to the invention, and

FIGS. 3A and 3B show schematically the densifying process of a plated grain.

it was compared with. However, it is difficult numerically to access the results. An attempt at such an assessment was however made in connection with the continued testing of the powder steel specimen (a) for an additional twenty days. A powder steel specimen (d) with a composition corresponding to (a) but without barriers was also tested simultaneously. Table 2 below shows this numerical comparison expressed as an "index of corrosion resistance" and based on the relation between the time and the maximum depth of cracks. The powder steel (a) with barriers showed a higher corrosion resistance than the steels (b) and (c). As compared with steel (b) the resistance was 5 times as high and as compared with steel (c) 3 times as high.

TABLE 2.—TRANSCRYSTALLINE STRESS CORROSION  
[Testing according to Table 1]

| Quality | Time until the first crack appeared | Test broken off after— | Maximum depth of cracks | Time elapsed until appearance of crack of a depth of 1.5–1.6 mm. | Index of corrosion resistance |
|---------|-------------------------------------|------------------------|-------------------------|------------------------------------------------------------------|-------------------------------|
| (a)     | 11 days                             | 35 days                | 1.6 mm                  | 35 days                                                          | 1.4                           |
| (b)     | 1 day                               | 11 days                | 2.5 mm                  | 7 days <sup>1</sup>                                              | 0.2                           |
| (c)     | 1 day                               | 11 days                | 1.5 mm                  | 11 days                                                          | 0.0                           |
| (d)     | 7 days                              | 13 days                | 1.6 mm                  | 13 days                                                          | 0.3                           |

<sup>1</sup> Approximate value assuming a linear function.

### EXAMPLES

A stainless austenitic steel composed of 0.06% C, 17.0% Cr, 9.3% Ni and balance Fe in powder form with a grain size of  $-1.17 \pm 0.1$  mm. was electrolytically plated with 4.3% Ni calculated on the total weight of the plated material. The powder was enclosed in a casing of non-alloyed steel, heated in a furnace at 1200° C. for 15 minutes and forged out to sheet metal with a thickness of 4 mm. and with a reduction of 1:5. The sheet metal was freed from the protective coating by means of pickling in nitric acid and hydrofluoric acid.

A stress corrosion test was carried out in the following way. A test specimen (specimen (a) in the table below) was cut out, formed to a size of 3 x 20 x 150 mm., cold-bent over a mandrel with a radius of 7.5 mm. and fastened to a holder that covered a 25 mm. portion of the specimen. The test specimen was immersed in a 40 percent  $\text{CaCl}_2$  solution at pH 6 and 100° C.

For the sake of comparison two standard materials rolled from cast ingots were corrosion tested in the same way. The one steel (b) retained a nickel content which corresponded fairly well to the basic content of the powder steel, while the other (c) corresponded approximately to the powder steel as to its average content of nickel.

After completing the test the test specimens were cut in a longitudinal direction in the places where the largest cracks had appeared, the greatest depth of the cracks was then measured and in certain cases micro-photographed.

The results of the test are shown in Table 1 below.

It was startling to find that the powder steel (d) without barriers had a resistance that was higher than that of steel (b) with a similar analysis with which it has compared, or to be more specific twice as high.

The time elapsed until the appearance of the first crack also gives an indication of the corrosion resistance. The dispersion of the results is usually rather wide in this test and that is why the results according to Table 1 and Table 2 ought to be considered with a certain caution. However, it is quite obvious that steel (a) yielded better results than the steels it was compared with. It is surprising that even steel (d) yielded better results than steels (b) and (c).

FIG. 1 is a microphoto of the cracks in steel (a) with barriers after a 15 days' test in a chloride solution. It shows how from the surface the cracks have forced their way down into the material to be blocked there by the first barrier, except in one point where the barrier was broken through. The crack front has then been caught by the next barrier.

In the course of a microsecond examination the nickel contents of the barriers varied between 20 and 60 percent, the lower content in the thin barriers and the higher content in the thick ones. By the heat treatment, for instance in connection with the plastic working, nickel diffuses from the barriers out into the basic material while a corresponding diffusion of iron, chromium and the other alloying elements present in the basic material takes place in the opposite direction.

The diffusion process is schematically shown in FIG. 2, where the left-hand Part I is meant to show a barrier

TABLE 1.—TRANSCRYSTALLINE STRESS CORROSION, U-SHAPED SPECIMENS

Solution: 40 percent  $\text{CaCl}_2$ , pH 6, 100° C.  
Specimen sizes: 3 x 20 x 150 mm.

| Quality                                                                                              | Time until the first crack appeared | Test broken off after— | Surface of specimen after—                                      |                         | Maximum depth of cracks after completed test |
|------------------------------------------------------------------------------------------------------|-------------------------------------|------------------------|-----------------------------------------------------------------|-------------------------|----------------------------------------------|
|                                                                                                      |                                     |                        | 11 days                                                         | Completed test          |                                              |
| (a) Powder steel according to the invention: 17 percent Cr, 9.3+4.3=13.6 percent Ni, 0.06 percent C. | 11 days                             | 15 days                | Single short (5 mm.) cracks.                                    | 6 short (5 mm.) cracks. | 0.32 mm.                                     |
| (b) Conventional steel: 18 percent Cr, 10.2 percent Ni, 0.4 percent Mo, 0.044 percent C.             | 1 day                               | 11 days                | Great number of cracks across the entire width of the specimen. | See preceding column.   | 2.50 mm.                                     |
| (c) Conventional steel: 16.6 percent Cr, 14.8 percent Ni, 4.3 percent Mo, 0.047 percent C.           | 1 day                               | 11 days                | Number of 10 mm. long cracks.                                   | do                      | 1.52 mm.                                     |

As is evident from the corrosion test, the powder steel (a) produced far better results than the specimens

with contiguous basic material prior to diffusion and the right-hand Part II the same material after diffusion.

The two upper part figures marked A (A(I) and A(II) respectively) show—on a greatly magnified scale—the same part section through two contiguous grains 1 with intervening barrier 2. Barrier 2 has been formed by adjoining two coated grains, the intermediate surface between these grains is indicated by dash-dotted line 4. The interface between the grains and the coating is marked 5. Part figure A(II) to the right illustrates the principle of how the diffusion changes the composition. The basic material of the grains (austenitic stainless steel) has penetrated into barrier 2 and the barrier material has penetrated into the basic material, a condition illustrated by the extension of the respective sectioning lines. In this way interface 5 has been erased but its former position is indicated by dash-dotted lines 5. Thus, areas 3 containing sectioning lines with two different inclinations consist of materials with composition gradients, i.e. increasing or decreasing contents of the chemical elements present in the basic material and the barrier.

The two central part figures marked B (B(I) and B(II)) as well as the two bottom part figures marked C (C(I) and C(II)) are meant to illustrate the composition of an arbitrary cross section through the section shown in part figures A(I) and A(II).

According to the embodiment of the invention shown in B(I) and B(II), austenitic stainless steel is coated with nickel. Basic material 1 contains about 70 percent Fe, 20 percent Cr and 10 percent Ni, barrier material 2 contains 100 percent Ni. The vertical dash-dotted and dashed lines showing the iron and chromium contents respectively in interface 5 have been displaced in parallel for the sake of clarification. As a matter of fact the lines for Fe, Cr and Ni coincide in interface 5, since no diffusion has taken place when the grains were coated. Part figure B(II) shows how the iron content decreases towards the barrier with a lowest value of about 43 percent Fe in the centre of the barrier. The Cr content decreases in the same way and reaches a lowest value of about 7 percent in the centre of the barrier. Contrarywise the Ni content increases and reaches the highest value of about 50 percent in the centre of the barrier. As was done in part figure A(II), the former position of interface 5 has been indicated by dash-pointed line 5.

For the plating of the powder material not only nickel may be used, but also nickel in combination with chromium, molybdenum, silicon, titanium, manganese and/or copper. The total amount of plated metal may reach 1 to 10 percent calculated on the powder weight preferably however 2 to 6 percent.

The plating of the powder material may be carried out by conventional plating methods such as, for instance, electrolytically, via volatile metal compounds (halides, carbonyls) and by means of evaporation—sublimation.

In case one wishes to add other metals besides nickel these may be applied simultaneously or one at a time. It is usually appropriate to coat the outside of the metal grains with nickel which has a low oxygen affinity. This method offers considerable advantages in connection with the heating and handling of the powder up to the stage where the material is available in a compact shape and is no longer so sensitive to oxidation. If, for instance, a powder in whose surface there is a higher concentration of chromium is to be heated to say 1150° C., this heating must be conducted in high vacuum in a very pure inert gas atmosphere or in hydrogen gas with an  $H_2/H_2O$ -ratio of a minimum of  $5 \cdot 10 \cdot 10^3 : 1$  if there is to be no oxidation. If, on the other hand, the powder surface has been plated with a layer of nickel, the question of the protective gas is very simple since the corresponding  $H_2H_2O$ -ratio only needs to reach a minimum of  $10^{-2} : 1$ . Even nitrogen gas may be used as a protective gas or a protective gas component, since at the above temperature there is no risk for the nickel of nitride formation.

According to the embodiment in part figures 2C(I) and 2C(II) the grains have first been gas chromi-

plated and subsequently nickel-plated. Here the object of the added chromium is to give the barriers a chromium content approximately corresponding to the chromium content in the basic material and thus give it general corrosion properties of an equal value.

The composition of the basic material is about 70 percent Fe, 20 percent Cr and 10 percent Ni. In the process of gas chromium-plating a diffusion takes place whereby the composition of the basic material in the surface layer is changed to about 35 percent Cr, about 57 percent Fe and about 8 percent Ni. After the nickel-plating of the grains and the diffusion treatment the composition changes once more in a way which is analogous to the embodiment according to part figures 2B. Thus the Fe content decreases to about 32 percent and the Cr content to about 18 percent in the centre of the barrier while the Ni content increases to about 50 percent.

By means of this embodiment of the present invention barriers have been created which have a high resistance both to transcrystalline corrosion in a chloride environment and to general corrosion.

The basic material i.e. the powder material prior to plating shall be of an austenitic stainless steel type or an acid-proof steel type with a nickel content of from 5 to 15 percent and a chromium content of from 16 to 25 percent. In addition the steel may contain, say, molybdenum, manganese, silicon, titanium and/or copper.

The size of the powder particles may vary within a relatively wide range. Tests have been made with material 30—5 mm. +0.05 mm. The grain size should be adapted to the demands made on the final product. A coarse powder results in thicker barriers but a larger distance between the barriers as compared to a finely divided powder, when using an equal amount of plating metal. The particle size should preferably lie within the range —4 +0.1 mm.

In this connection the terms “—5 mm.” or “—4 mm.” imply that the material passes through a sieve with square sieve openings having a side of 5 or 4 mm. respectively.

In this connection the terms “+0.05 mm.” or “+0.1 mm.” imply that the material stays on a sieve with square sieve openings having a side of 0.05 or 0.1 mm. respectively.

In order to obtain dense surrounding layers in the process of plating the metal particles should not be of too irregular a shape and they should have smooth surfaces free from oxide and slag.

In order to obtain a 100 percent material density during the plastic working the reduction of the sectional area should be a minimum of 1:4. In this way one may also be sure that the barriers are given a suitable orientation, i.e. mainly parallel to the surfaces of the sheet metal or of the bar material and consequently mainly angular to the direction of the cracks.

By means of the above-mentioned reduction the barrier steel also achieves a strength corresponding to that of the basic material. The steel produced according to the present invention showed the following strength characteristics:

|    | Tensile strength |            | Elongation<br>percent |
|----|------------------|------------|-----------------------|
|    | $\sigma_{0.2\%}$ | $\sigma_B$ |                       |
| 65 | 29.9             | 63.9       | 56.2                  |
| 66 |                  |            | 45.5                  |

If the plated layer is softer and more plastic than the basic material at the relevant temperature for the densifying, a redistribution of the layer takes place in the course of the pressing and stretching of the particles. The process has been schematically illustrated in FIG. 3A, which shows a sectional view of grain 6 prior to densifying and the same grain marked 7 after densifying. The basic material of the grain is marked 8 and 9 respectively and the coating 10 and 11 respectively. The figure is intended

to show how a considerable accumulation of coating material has taken place at 12. The thickness of the barriers may thus vary within a wide range, with considerable accumulations of plated metal in certain areas and corresponding thinning in others. This process implies that the plating material is not so fully utilized. The situation may be improved if prior to plating the particles are formed according to FIG. 3B. The relation  $D/d$  may suitably be maintained within the range 1.5:1 to 4:1. The grains have been flattened in a way to make their shape resemble a disc or an ellipsoid.

What we claim is:

1. A process for the production of an austenitic stainless steel alloy having a high resistance to transcrystalline stress corrosion in a chloride environment afforded by corrosion-impeding barriers oriented in planes generally parallel to each other comprising the steps of forming on the individual particles of an austenitic stainless steel powder a plated coating virtually covering each particle of a corrosion-resistant material including predominantly nickel, the material being present in the coated powder in an amount by weight of from about 1% to about 10% based on the total weight, forming a body of the coated powder, sintering the said body, and compacting and permanently deforming the body by plastic working substantially to reduce the cross-sectional area of the body in a direction transverse to the said parallel planes and substantially to elongate the body in a direction aligned with the said parallel planes.

2. A process according to claim 1 wherein the cross-sectional area of the body is reduced to the extent that the final cross-sectional area is not greater than about

one-fourth of the original cross-sectional area of the body.

5 3. A process according to claim 1 wherein the coating material is present in the coated powder in an amount by weight of from about 2% to about 6% based on the total weight.

10 4. A process according to claim 1 wherein the coating material further includes a minor portion of at least one metal selected from the group consisting of chromium, molybdenum, silicon, titanium, manganese and copper.

15 5. A process according to claim 1 wherein the particles of the stainless steel powder pass a screen having square openings measuring 5 mm. and are retained on a screen having square openings measuring 0.05 mm.

15

#### References Cited

##### UNITED STATES PATENTS

|           |         |         |          |
|-----------|---------|---------|----------|
| 2,610,118 | 9/1952  | Drapeau | 75—212 X |
| 2,933,415 | 4/1960  | Homer   | 75—212 X |
| 3,223,523 | 12/1965 | Adler   | 75—212   |
| 3,310,870 | 3/1967  | Parikh  | 29—420.5 |

20

##### FOREIGN PATENTS

|           |        |         |
|-----------|--------|---------|
| 768,067   | 5/1934 | France. |
| 38/27,988 | 9/1963 | Japan.  |

25

CARL D. QUARFORTH, Primary Examiner

A. J. STEINER, Assistant Examiner

30

U.S. Cl. X.R.

75—214; 29—182.2, 420.5

UNITED STATES PATENT OFFICE  
CERTIFICATE OF CORRECTION

Patent No. 3,479,181 Dated November 18, 1969

Inventor(s) A. I. Backstrom et al.

It is certified that error appears in the above-identified patent and that said Letters Patent are hereby corrected as shown below:

Column 2, line 33, "Mineral" should be  
-- Material --;

Column 4, line 21, "1.4" should be -- 1.0 --;

Column 4, line 23, "0.0" should be -- 0.3 --;

Column 4, line 24, "0.3" should be -- 0.4 --;

Column 6, line 64, "S B" (second occurrence)  
should be -- ~~S~~5 --;

Column 6, line 65, "56.2" should be -- 56.4 --.

**SIGNED AND  
SEALED  
JUN 2 1970**

**(SEAL)**

**Attest:**

**Edward M. Fletcher, Jr.**

**Attesting Officer**

**WILLIAM E. SCHUYLER, JR.  
Commissioner of Patents**